# EUROPEAN PATENT SPECIFICATION

(11) **EP 3 006 611 B1**
(45) Date of publication and mention of the grant of the patent: **20.02.2019**
(21) Application number: 14808311.6
(22) Date of filing: 28.05.2014
(51) Int. Cl.: D02G 3/22, D07B 1/02, D07B 1/16, E04C 5/07, D06M 15/55, D07B 7/14, D04C 1/02, D02G 3/40

(54) **STRAND STRUCTURE, AND MULTI-STRAND STRUCTURE**
STRANGSTRUKTUR UND MEHRSTRANGIGE STRUKTUR
CORPS STRUCTUREL À BRINS AINSI QUE CORPS STRUCTUREL MULTIBRINS

(30) Priority: 05.06.2013 JP 2013119113
(43) Date of publication of application: 13.04.2016
(73) Proprietor: KOMATSU MATERE Co., Ltd., Nomi-City Ishikawa 929-0124 (JP)
(72) Inventor: HAYASHI, Yutaka, Nomi-City Ishikawa 929-0124 (JP); NAKAYAMA, Taketoshi, Nomi-City Ishikawa 929-0124 (JP); NODA, Honami, Nomi-City Ishikawa 929-0124 (JP)
(74) Representative: Winter, Brandl, Fürniss, Hübner, Röss, Kaiser, Polte - Partnerschaft mbB
(86) International application number: PCT/JP2014/064127
(87) International publication number: WO 2014/196432

(56) References cited:
- WO-A1-2006/043311
- WO-A1-2009/108200
- CN-A- 102 081 993
- JP-A- 2006 182 915
- JP-A- 2012 136 814
- JP-A- 2012 136 814
- JP-A- 2012 251 378
- JP-A- 2013 011 162
- JP-A- 2013 213 305
- JP-U- H03 125 089
- US-A1- 2008 028 740
- US-A1- 2008 282 664
- US-A1- 2011 192 132

## Description

### FIELD OF THE INVENTION

The invention relates to a strand structure including a strand construction comprised of two or more twisted high-strength fiber composites, each including a core comprised of bundled high-strength fiber yarns, the bundle being twisted and stiffened with a stiffening agent.

### BACKGROUND ART

A carbon fiber is excellent in physical properties such as a tensile strength and an elastic modulus, and a resistance to corrosion caused by acid and alkali, and further, is lightweight. Consequently, a carbon fiber is employed in various fields in industries such as an automobile, an airplane, electric/electronic devices, a toy, and domestic appliances, and is attempted to be applied to architectures. For instance, the patent document 1 suggests an example in which a carbon fiber composite is employed as a tensile member of a brace in a frame in order to enhance earthquake-proof of a building. Furthermore, the patent document 2 suggests an example of a wire made of carbon fiber composites. Patent document 2 discloses the features of the preamble of claim 1.

A carbon fiber composite is able to enhance a tensile strength and a bending strength, but is accompanied with a problem of being weak against a shearing force. This problem is found not only in a carbon fiber yarn, but also in a high-strength fiber composite fabricated by bundling fibers called high-strength fibers such as basalt fiber yarns in a common direction to thereby fabricate a high-strength fiber bundle, and covering the thus fabricated high-strength fiber bundle at an outer surface thereof with another fiber.

In addition, the inventors have reported, in the patent document 3, a high-strength fiber composite (a cord-shaped reinforced fiber composite) including an internal layer comprised of a core composed of one or more bundle(s) of cord-shaped carbon fibers, an intermediate layer including resin surrounding the core, and an external layer comprised of a cylindrically knit cord surrounding the intermediate layer. The high-strength fiber composite has a superior tensile strength derived from carbon fibers, a superior shearing strength, and is able to change a shape thereof in the preferred embodiment of the high-strength fiber composite.

On the other hand, in the case that a bending stress is exerted onto the high-strength fiber composite, for instance, when the high-strength fiber composite is wound by means of a wire or a rope around a drum having a small diameter, the carbon fiber bundles defining the core of the high-strength fiber composite are sometimes partially broken, resulting in that a tensile strength of the high-strength fiber composite at an entirety thereof is afraid to be deteriorated. Furthermore, in the case that the high-strength fiber composite is employed as a rod of a tensile member, the high-strength fiber composite is afraid to be accompanied with the above-mentioned problem, because the high-strength fiber composite having a great length is sometimes stored in such a condition as being wound around a drum.

### PRIOR ART DOCUMENTS

### PATENT DOCUMENTS

Patent document 1: Japanese Patent Application Publication 2006-348506
Patent Document 2: United States Patent Application Publication 2008/0028740
Patent Document 3: Japanese Patent Application Publication 2012-136814

### SUMMARY OF THE INVENTION

### PROBLEM(S) TO BE SOLVED BY THE INVENTION

As mentioned above, a high-strength fiber composite comprised of a bundle of high-strength fibers fabricated by twisting high-strength fiber yarns such as carbon fiber yarns is accompanied with a problem that when the high-strength fiber composite is used under a bending stress, for instance, when the high-strength fiber composite is used as a wire or a rope, or when the high-strength fiber composite is stored in a condition of being wound around a drum, the high-strength fiber composite is sometimes not able to sufficiently provide superior inherent performances of high-strength fiber yarns, and thus, there is a need for improvement.

In view of the above-mentioned problem in the conventional high-strength fiber composite, it is an object of the present invention to provide a high-strength fiber composite capable of having an inherent tensile strength of high-strength fiber yarns, even when the high-strength fiber composite is used under a bending stress, and to provide products to which the high-strength fiber composite is applied.

### SOLUTION TO THE PROBLEM(S)

The present invention provides a strand structure according to claim 1, and a multi strand structure comprising the strand structure according to the invention.

Preferred embodiments of the strand structure and multi strand structure are defined in the appended claims.

Namely, an aspect of the disclosure relates to a high-strength fiber composite including a core comprised of a bundle of high-strength fiber yarns, the bundle being twisted and stiffened with a stiffening agent.

In the above-identified high-strength fiber composite, since the core defining the high-strength fiber composite is stiffened with a stiffening agent in a condition that the bundle of high-strength fiber yarns are twisted, even if an external intensive force acts on the high-strength fiber composite, it is possible to prevent the high-strength fiber yarns defining the high-strength fiber bundle from being untied from one another, ensuring that the high-strength fiber yarns can stably have an inherent tensile strength thereof.

Furthermore, since the high-strength fiber yarns defining the high-strength fiber bundle are not untied from one another because the high-strength fiber bundle is stiffened with a stiffening agent in a condition that the bundle of high-strength fiber yarns are twisted, the high-strength fiber composite can have enhanced (stabilized) handling property and strength, and the high-strength fiber yarns are hardly broken even if bent. If the high-strength fiber bundle is not twisted, the high-strength fiber composite may be broken in the case that the high-strength fiber composite is wound around a drum, or that the high-strength fiber composite is employed in such a condition that a bending stress acts thereon. Consequently, it is afraid that the high-strength fiber composite (and accordingly, a later-mentioned strand structure comprised of the high-strength fiber composite) cannot be employed, and cannot have an inherent strength of the high-strength fiber yarns. In addition, if the high-strength fiber bundle is not twisted, there may occur fluctuation in a length of each of the high-strength fiber yarns in the high-strength fiber bundle, the high-strength fiber bundle cannot have an inherent strength of a high-strength fiber which each of the high-strength fiber yarns have, resulting in that the high-strength fiber bundle may be short in a strength as an entirety thereof.

By imparting twist to the high-strength fiber bundle, it is possible to prevent the high-strength fiber composite from being broken, and the high-strength fiber yarns defining the high-strength fiber bundle can have a uniformized length, ensuring an inherent strength of a high-strength fiber. Thus, the high-strength fiber composite can keep an intensive tensile strength, even if a bending stress acts thereon, specifically, when the high-strength fiber composite is stretched after having been wound around a drum, or when the high-strength fiber composite is pulled with the high-strength fiber composite being kept bent.

If the high-strength fiber bundle is merely twisted without being stiffened with a stiffening agent, the resultant high-strength fiber composite can have a strength smaller than the same of the high-strength fiber composite in accordance with the present invention in which the high-strength fiber bundle is stiffened with a stiffening agent.

The high-strength fiber composite may be designed to include any one of high-strength fibers to be described later in the embodiments. It is preferable for the high-strength fiber to include basalt fibers or carbon fibers, and more preferable to include carbon fibers. Accordingly, it is preferable for the high-strength fiber yarns defining the high-strength fiber bundle to include carbon fibers or basalt fibers, more preferable to be carbon fibers or basalt fibers, and particularly preferable to be carbon fibers.

Basalt fiber and carbon fiber have a high tensile strength, but have a low shearing strength, and accordingly, are easy to be broken. Consequently, in the case that a high-strength fiber composite including basalt fibers or carbon fibers are used under a bending stress, for instance, a high-strength fiber composite is used as a wire or a rope, or stored in a condition of being wound around a drum, the high-strength fiber composite is easy to be broken. However, by imparting twist to a high-strength fiber bundle comprised of basalt fibers or carbon fibers, a high-strength fiber composite can be prevented from being broken even if a force acts thereon in a direction perpendicular to a length-wise direction of the high-strength fiber composite. Thus, the high-strength fiber composite including a high-strength fiber bundle comprised of basalt fibers or carbon fibers is able to have an inherent tensile strength of basalt fiber or carbon fiber, even if a bending stress acts thereon.

The high-strength fiber composite includes a constraint wound around the high-strength fiber bundle, the high-strength fiber bundle and the constraint being stiffened together with the stiffening agent with the high-strength fiber bundle being kept twisted, to define the core.

By winding a constraint around the twisted high-strength fiber bundle to thereby tie high-strength fibers together, and further by stiffening the high-strength fiber bundle and the constraint together with a stiffening agent to thereby define a core, it is possible to prevent high-strength fiber yarns defining the high-strength fiber bundle from being twisted, crossed and/or untied from one another, even if an external intensive force acts thereon, ensuring that the high-strength fiber composite is able to keep having a tensile strength inherent to high-strength fibers. By using twisted high-strength fiber bundle, the high-strength fiber composite can be prevented from being broken after being stiffened with a stiffening agent, even if a bending stress acts thereon.

Any constraint can be used, if it can be wound around a high-strength fiber bundle to thereby keep the high-strength fiber bundle twisted. In particular, it is preferable that a constraint covers an entire circumference of a high-strength fiber bundle therewith. By covering entirely circumferentially a high-strength fiber bundle (in particular, carbon fibers or basalt fibers) with a constraint, it is possible to obtain the above-mentioned advantages, and further possible to prevent the high-strength fiber yarns from being cut, even if the high-strength fiber makes contact with sharpened materials such as pebbles.

The constraint for bundling the high-strength fiber bundle has a braid structure, because the high-strength fiber bundle can be covered therewith to such a degree that a surface of the high-strength fiber bundle is not visible with eyes, and accordingly, the constraint not only bundles the high-strength fiber bundle, but also acts as a protection layer for protecting high-strength fiber yarns of which the internal high-strength fiber bundle is comprised.

If the high-strength fiber bundle is not twisted, the high-strength fiber yarns defining the high-strength fiber bundle sometimes spring out beyond the constraint before being stiffened with a stiffening agent. By employing a twisted high-strength fiber bundle, it is possible to prevent the high-strength fiber yarns defining the high-strength fiber bundle from being twisted, crossed, untied, broken and/or cut, even if an external intensive force acts thereon, ensuring that it is possible to maintain handling property of the high-strength fiber bundle even before the high-strength fiber bundle is stiffened with a resin, and hence, the high-strength fiber composite can sufficiently have an inherent tensile strength thereof.

A number of twisting the high-strength fiber bundle is preferably in the range of 2 to 50 times per a meter both inclusive, and more preferably in the range of 4 to 40 times per a meter both inclusive. The number is preferably is equal to or greater than 10 times per a meter, more preferably is equal to or greater than 15 times per a meter, and most preferably is equal to or greater than 20 times per a meter. The upper limit of the number is equal to or smaller than 50 times per a meter, and preferably is equal to or smaller than 40 times per a meter. If the number of twisting the high-strength fiber bundle is smaller than 2 times per a meter, the advantages obtained by twisting the high-strength fiber bundle are afraid of turning insufficient, and if the number is greater than 50 times per a meter, the high-strength fiber yarns defining the high-strength fiber bundle are afraid of being cut during being twisted.

As the stiffening agent a thermoplastic resin is used, because it can be readily thermally deformed, can be readily wound around a thin drum while being heated, and can readily form a later-mentioned strand structure. Furthermore, it is preferable for the stiffening agent to have high affinity with the high-strength fiber yarns.

The stiffening agent will be explained in detail in the later-mentioned embodiments. It is preferable to select as a thermoplastic resin a thermoplastic epoxy resin (in particular, a thermoplastic epoxy resin having a straight-chain shaped polymeric structure). Among thermoplastic epoxy resins, it is preferable to employ a polymerization type thermoplastic epoxy resin (in particular, a thermoplastic epoxy resin having a straight-chain shaped polymeric structure).

It is preferable in the high-strength fiber composite that the core has a diameter in the range of 1 to 5 mm both inclusive. A diameter of the core is defined as the greatest diameter among diameters of portions of the high-strength fiber composite. The constraint is included in a diameter of the core.

By designing the core to have a diameter in the above-identified range, it is possible to wind the high-strength fiber composite around a drum having a small diameter (for instance, a drum having a diameter equal to or smaller than 70 cm), without heating the high-strength fiber composite. Furthermore, a strand structure comprised of the high-strength fiber composites can be readily wound around a drum having a small diameter, and the strand structure would have a large area when the strand structure is adhered at an end thereof to a jig for fixation, ensuring contribution to enhancement in an adhesion strength of the strand structure with the jig.

Furthermore, the high-strength fiber includes at least the above-mentioned core, and may be colored at an outer surface thereof, and/or may further include a protection layer covering an outermost layer therewith.

According to the present invention, there is provided a strand structure including a strand construction comprised of two or more twisted high-strength fiber composites whereby each of the twisted high-strength fiber composites includes a core comprised of a bundle of high-strength fiber yarns, the bundle being twisted and stiffened with a stiffening agent,each of the twisted high-strength fiber composites further includes a constraint wound around the bundle, the bundle and the constraint being stiffened together with the stiffening agent with the bundle being kept twisted, to define the core,the constraint forms a cylindrical braid of winded fibers, and the stiffening agent is composed of thermoplastic resin.

Herein, "a strand construction" means a construction comprised of two to tens of strands twisted together in a single layer or a plurality of layers, the strands having a common diameter of diameters different from one another.

Since the strand structure in accordance with the present invention is comprised of the high-strength fiber composites having the above-mentioned properties, the strand structure can act as a composite maintaining the above-mentioned performances of the high-strength fiber composite, and further, being superior in a tensile strength.

A strand structure in accordance with the present invention can be fabricated by drawing elongate high-strength fiber composites out of a creel by a requisite number, and twisting them. Because a thermoplastic resin is used as the above-mentioned stiffening agent, it is preferable that the high-strength fiber composites are twisted while being heated at a temperature at which the thermoplastic resin is softened.

The thus fabricated strand structure is elongate, and can be stored in such a condition as being wound around a drum, similarly to the high-strength fiber composite. The strand structure is cut into pieces having a suitable length, and can be used as a wire, a rope, and so on. As an alternative, the strand structure may be cut into a rod-shape, and can be used as a reinforcing bar of concrete or a tensile member.

By being twisted, the resultant strand structure can be wholly tied with one another, ensuring is possible to prevent the strand structure from being untied from one another, and further ensuring that a tensile strength thereof can be maintained stable.

The strand structure in accordance with the present invention includes the high-strength fiber composites by two or greater. A number of the high-strength fiber composites to be included in the strand structure is determined in dependence on target performances (in particular, a tensile strength) and an intended use thereof. The number is generally in the range of 2 to 40 both inclusive, and preferably in the range of 7 to 37 both inclusive. If the number is greater than 40, it is afraid that it is difficult to twist the strand structure at a predetermined pitch.

A process of twisting the strand structure in accordance with the present invention may include steps of (1) bundling a requisite number of the high-strength fiber composites, and imparting twist wholly to the thus bundled high-strength fiber composites, or (2) centrally arranging a single or a plurality of the high-strength fiber composite(s) as a core, arranging other high-strength fiber composites to surround the core high-strength fiber composite(s), and imparting twist to the core high-strength fiber composite(s) and the other high-strength fiber composites together.

It is preferable that a number of twisting the strand structure in accordance with the present invention is in the range of 1.1 to 50 times per a meter both inclusive, regardless of whether the above-mentioned steps (1) or (2) are carried out. In particular, in the case that a number of the high-strength fiber composites defining the strand structure is in the range of 7 to 37 both inclusive, a number of twisting the strand structure is preferably in the range of 1.5 to 20 times per a meter.

In a further aspect, there is provided a multi-strand structure including a strand construction comprised of two or more twisted strand structures, each strand structure being in accordance with the present invention. Herein, "a multi-strand construction" means a construction in which the strand structure in accordance with a second aspect of the present invention is used as a strand, and two to tens of strands (the strand structures) are twisted in a single layer or a plurality of layers, the strands having a common diameter with one another or having different diameters from one another.

By designing the strand construction (the multi-strand construction) to be comprised of twisted strand structures, as mentioned above, the resultant multi-strand construction can have a greater strength than a strand construction merely including strand structures by the same number. Thus, the multi-strand structure is useful particularly for a case that a high tensile strength is required, such as a reinforcing bar, a PC steel wire, or a PC steel member to be used in a big building, and a wire to be used in place of chains for mooring a big vessel.

The multi-strand structure in accordance with the present invention has advantages in having good handling property, because the strand structures defining the multi-strand structure are more difficult to be untied from one another than a multi-strand structure merely including the strand structures by the same number, and further, in having a stable strength.

A number of the strand structures (in accordance with the present invention) to define the multi-strand structure in accordance with the present invention is at least two, and is determined in dependence on required performances (in particular, a tensile strength) and uses thereof. The number is generally in the range of 2 to 40 both inclusive. If a number of the strand structures for defining the multi-strand structure is greater than 40, it is afraid to be difficult to twist the strand structures at a predetermined pitch. The number is preferably in the range of 7 to 37 both inclusive.

A process of twisting the multi-strand structure in accordance with the present invention may include steps of (1) bundling a requisite number of the strand structures, and imparting twist wholly to the thus bundled strand structures, or (2) centrally arranging a single or a plurality of the strand structure(s) as a core (hereinafter, called "core strand"), arranging other strand structures to surround the core strand, and imparting twist to the core strand and the other strand structures together.

It is preferable that a number of twisting the multi-strand structure in accordance with the present invention is in the range of 0.3 to 30 times per a meter both inclusive, regardless of whether the above-mentioned steps (1) or (2) are carried out. In particular, in the case that a number of the strand structures defining the multi-strand structure is in the range of 7 to 37 both inclusive, a number of twisting the multi-strand structure is preferably in the range of 0.5 to 15 times per a meter.

The strand structure in accordance with the present invention, and the multi-strand structure in accordance with the present invention are applicable to all industrial fields such as civil engineering works, architecture, construction, vessel, mining and fishery, and are not to be limited with respect to an intended use thereof.

The strand structure, and the multi-strand structure all in accordance with the present invention have a superior strength derived from high-strength fibers, and are lightweight, they can be preferably used in an architecture such as a steel skeleton construction, reinforced concrete, and a wooden building, and further in a brace member and a reinforcing member (including being used as a replacement of a reinforcing metal) both used as a bridge. Furthermore, since they have a sufficient strength, even though they are thin, they can be used in various items, for instance, a wire for suspending a furniture such as a light or a table, or a step, an interior such as a partition, a table, a chair, and a hand rail, a fence, a wall, an ivy support used for a green wall, and an exterior such as a net, ensuring fabrication of a building being superior in a design. In addition, they are useful as a replacement with chains used for mooring a vessel or a facility for carrying out wind power generation on a sea, both being likely to be suffered from salt damage. Furthermore, since they are difficult to be broken, even if a bending stress acts thereon, they can be preferably used as a long one by wind them around a drum, or used under a bending stress environment.

The strand structure, and the multi-strand structure all in accordance with the present invention may be colored at an outer surface thereof, or may be designed to further include a protection layer as an outermost layer.

Furthermore, the strand structure or the multi-strand structure in accordance with the present invention may be compounded with any other item into a compound-structure item. As a preferable compound-structure item, there is provided a compound-structure item including the strand structure or the multi-strand structure and a jig, wherein the strand structure or the multi-strand structure is inserted through at least one of ends thereof into a body of the jig, and then, the strand structure or the multi-strand structure is fixedly adhered at the end to the body of the jig to thereby define a compound-structure item in which the strand structure or the multi-strand structure and the jig are joined into one piece.

As a preferable jig to be compounded with a high-strength fiber composite in accordance with the present invention, there was suggested the jig by the inventors in Japanese Patent Application No. 2012-84240. Since the twisted high-strength fiber composites are not bundled by means of a stiffening agent in the case that the strand structure is used as a reinforcing bar in concrete, the strand structure can have an increased surface area to thereby have an increased contact strength with concrete, ensuring an increase in a strength of a concrete architecture and so on.

### ADVANTAGES PROVIDED BY THE INVENTION

Providing a high-strength fiber composite having an inherent tensile strength of high-strength fibers, and being capable of being preferably used under a bending stress environment. The high-strength fiber composite in accordance with the present invention has advantages that it can be used in a bending stress environment, for instance, in the case that it can be used as a wire or a rope, and that a strength thereof is difficult to be reduced even if it is stored in such a condition as being wound around a drum.

Furthermore, a strand structure and a multi-strand structure in accordance with the present invention have a strength derived from high-strength fibers, and are lightweight and superior in a tensile strength, ensuring that they can be used for various purposes.

### BRIEF DESCRIPTION OF THE DRAWINGS

FIG. 1 is an illustration of the high-strength fiber composite in accordance with a first embodiment.
FIG. 2 is an illustration of a process of fabricating the high-strength fiber composite.
FIG. 3A is an illustration (a side view) of the high-strength fiber composite 1a in accordance with a second embodiment.
FIG. 3B is an illustration (a cross-sectional view) of the high-strength fiber composite 1a in accordance with the second embodiment.
FIG. 4 is an illustration of the strand structure 10 in accordance with a third embodiment which falls under the scope of the present invention.
FIG. 5A is an illustration (a side view) of the multi-strand structure 100 in accordance with a fourth embodiment which falls under the scope of the present invention.
FIG. 5B is an illustration (a cross-sectional view (seven strand structures 10)) of the multi-strand structure 100 in accordance with the fourth embodiment which falls under the scope of the present invention.
FIG. 6 is a photograph of the high-strength fiber composite in accordance with the first embodiment.
FIG. 7 is a photograph of the strand structure (a pitch of twisting: 20 times per a meter) in accordance with the third embodiment.
FIG. 8 is a photograph of the strand structure (a pitch of twisting: 5 times per a meter) in accordance with the fourth embodiment.
FIG. 9 is a photograph of the multi-strand structure in accordance with the fifth embodiment.

### INDICATION BY REFERENCE NUMERALS

1, 1a High-strength fiber composite
1b High-strength fiber composite acting as a core
1c High-strength fiber composites surrounding the high-strength fiber composite acting as a core
2 Core
3 Constraint
4 High-strength fiber yarn
5 High-strength fiber bundle
7a Creel
7b Dice
7c Heating furnace
7d Roller
7e Drum
7g Pre-heating furnace
7f Dice
10 Strand structure
10a Strand structure acting as a core (Core strand)
10b Strand structures surrounding Core strand
100 Multi-strand structure

### EMBODIMENTS FOR REDUCING THE EMBODIMENTS TO PRACTICE

Embodiments of the strand structure in accordance with the present invention are explained hereinbelow with reference to drawings. It is to be understood that the subject matter encompassed by way of the present invention is not to be limited to those specific embodiments, and that it is intended for the subject matter of the present invention to include all alternatives, modifications and equivalents as can be included within the scope of the following claims. In the specification, the expression "the range A to B" means that A and B are both inclusive in the range.

### (First Embodiment)

FIG. 1 illustrates a high-strength fiber composite 1 in accordance with the first embodiment which does not fall under the scope of the present invention. The high-strength fiber composite 1 includes a core 2 comprised of a twisted high-strength fiber bundle 5 stiffened by means of a stiffening agent.

The high-strength fiber bundle 5 is comprised of a plurality of high-strength fiber yarns 4 (generally, thousands of to hundred thousands of high-strength fiber yarns, or millions of high-strength fiber yarns) bundled with one another, and has a circular or oval cross-section. The high-strength fiber composite 1 in accordance with the first embodiment is stiffened by means of a stiffening agent with the high-strength fiber bundle 5 being twisted by a predetermined number. A number of twisting the high-strength fiber bundle 5 is determined in dependence on a resistance of a resultant high-strength fiber composite to a bending stress, property of preventing the high-strength fiber yarns from being unbundled, and a strength of the high-strength fiber yarns 4 against being twisted (the high-strength fiber yarns are not broken even by being twisted), and further determined such that carbon fiber bundle does not spring out of a constraint when bound by the constraint before being stiffened with a later-mentioned stiffening agent. A number of twisting the high-strength fiber bundle 5 is preferably in the range of 2 to 50 times per a meter both inclusive., more preferably in the range of 5 to 40 times per a meter both inclusive, and most preferably in the range of 10 to 30 times per a meter both inclusive.

The core 2 in the high-strength fiber composite 1 has a diameter preferably in the range of 1 to 10 mm both inclusive, and more preferably in the range of 1 to 5 mm both inclusive. In the first embodiment, a diameter of the high-strength fiber composite 1 is defined as a total of a diameter of the high-strength fiber bundle 5 and a thickness of a stiffening agent. A diameter of the high-strength fiber bundle 5 and an amount of a stiffening agent are determined such that the high-strength fiber composite 1 can have a target diameter.

By designing the core to have a diameter in the range of 1 to 10 mm both inclusive (preferably, in the range of 1 to 5 mm both inclusive), the high-strength fiber composite, a later-mentioned strand structure, and a later-mentioned multi-strand structure can be readily wound around a drum, and can have flexibility sufficient to follow an arbitrary shape. Furthermore, by designing the core to have a diameter in the range of 1 to 10 mm both inclusive (preferably, in the range of 1 to 5 mm both inclusive), a strand structure and a multi-strand structure can have a large surface area with a jig when they are adhered at an end thereof to the jig, ensuring enhancement in an adhesion strength between the jig and the strand structure or the multi-strand structure.

As the high-strength fiber yarn 4 defining the high-strength fiber bundle 5, there may be employed fiber sometimes called super fiber. As the high-strength fiber yarn 4, there may be employed, for instance, carbon fiber, basalt fiber, para-series aramid fiber, meta-series aramid fiber, polyethylene fiber having a super-high molecular weight, polyarylate fiber, PBO (polyparaphenylenebenzoxazole) fiber, polyphenylenesulfide (PPS) fiber, polyimide fiber, fluorine fiber, and polyvinyl alcohol (PVA) fiber. The high-strength fiber yarn 4 in the present invention may be comprised of carbon fiber or basalt fiber having a high strength in a direction in which fiber extends, but being weak against a shearing force. In particular, carbon fiber is useful as the high-strength fiber yarn.

The high-strength fiber bundle 5 may be defined with a single kind of the above-identified high-strength fiber yarn, or with a mixture of two or more kinds of the above-identified high-strength fiber yarns. The high-strength fiber bundle 5 may be designed to further include yarns comprised of organic fibers other than the above-identified high-strength fibers as long as a strength and/or a bending property thereof are (is) not deteriorated. Furthermore, the high-strength fiber bundle 5 may include a sizing agent and/or a bundling agent.

In the case that carbon fibers are employed as the high-strength fiber yarns 4 defining the high-strength fiber bundle 5, polyacrylonitrile (PAN)-series and pitch-series carbon fiber yarn may be employed. Among them, it is preferably to employ PAN-series carbon fiber yarn in the standpoint of a balance between a strength and an elastic modulus of a resultant product.

The high-strength fiber bundle fabricated by bundling the high-strength fiber yarns may be comprised of a single bundle or a plurality (two or more) of bundles of carbon fiber yarns in dependence on a required strength. The bundle may be comprised of 6000 carbon fiber yarns (6K), 12000 carbon fiber yarns (12K), 24000 carbon fiber yarns (24K), and so on, supplied from a carbon fiber manufacturer. A number of the high-strength fiber bundles in the case that a plurality of the high-strength fiber bundles each fabricated by bundling carbon fiber yarns is bundled is not to be limited to a particular number. The number is determined in dependence on a purpose and/or an intended use thereof, and is generally equal to or smaller than 100.

Any one of thermoplastic resin may be used as a stiffening agent. It is preferable that a stiffening agent has high affinity with the high-strength fiber yarn. A stiffening agent is comprised thermoplastic resin, because thermoplastic resin can be deformed when being heated.

As preferable examples of thermoplastic resin, there are polyetheretherketone (PEEK), polypropylene, polyethylene, polystyrene, polyamide (nylon 6, nylon 66, nylon 12, nylon 42, and so on), ABS resin, acrylate resin, vinyl chloride resin, vinylidene chloride resin, polyphenylene oxide, polybutylene terephthalate, polyethylene terephthalate, polysulfone, polyethersulfone, polyetherimide, polyarylate, epoxy resin, urethane resin, polycarbonate resin, resorcinol resin, and so on. Thermoplastic resin is not to be limited to the above-mentioned ones.

Among the above-identified resins, it is preferable in a standpoint of a durability against acid and alkali to use polyetheretherketone (PEEK), acrylic resin, vinyl chloride resin, vinylidene chloride resin, polyethylene resin, epoxy resin, urethane resin, polycarbonate resin, and resorcinol resin. It is particularly preferable to use epoxy resin, because it is superior in a resistance to impact. Furthermore, since thermoplastic epoxy resin is soluble in ketone solution, it can be divided from other resins, and hence, be recycled.

It is preferable to employ, among thermoplastic epoxy resins, polymerization type thermoplastic epoxy resin capable of formulating polymer, and more preferably to employ polymerization type thermoplastic epoxy resin capable of formulating polymer in a straight-chain shape.

If the high-strength fiber bundle defining a core were twisted, and/or if the high-strength fiber bundle were covered with a constraint, it would be difficult to allow resin to be impregnated into the high-strength fiber bundle.

In contrast, it is easy to control a viscosity of polymerization type thermoplastic epoxy resin, because thermoplastic epoxy resin before being polymerized can be diluted with organic solvent.

Accordingly, it is possible to allow thermoplastic epoxy resin before being polymerized to penetrate the twisted high-strength fiber bundle (furthermore, the high-strength fiber bundle through a constraint with which the high-strength fiber bundle is covered even in the case of the high-strength fiber bundle which is covered with a constraint) by means of resin solution having a low viscosity and being diluted with organic solvent. After thermoplastic epoxy resin before being polymerized was allowed to be impregnated into the high-strength fiber bundle, the polymerization type thermoplastic epoxy resin is polymerized to thereby obtain the high-strength fiber composite including the high-strength fiber bundle and the constraint both joined together through thermoplastic epoxy resin, and having a superior strength.

General thermoplastic rein used by being heated to be molten to thereby provide fluidity thereto is difficult to be controlled with respect to a viscosity thereof, and is afraid that arrangement of crystal thereof is varied by being heated and molten, because thermoplastic resin is generally crystalline, and hence, inherent properties thereof such as a strength may be deteriorated. In contrast, since polymerization type thermoplastic epoxy resin is amorphous before and after being polymerized, polymerization type thermoplastic epoxy resin has small risk against deterioration even by being heated to be molten or by heated to be deformed.

A process of applying the above-mentioned resin (a stiffening agent) to the high-strength fiber bundle 5 may include steps of coating by spraying or coating the resin onto high-strength fibers with a brush, but, on a standpoint of productivity, preferably includes step of dip-nipping or steps of dipping the high-strength fibers into resin (a stiffening agent) solution, and squeezing excessive resin through a dice. As a preferable example of an apparatus for applying resin (a stiffening agent) to the high-strength fiber bundle, there is an apparatus illustrated in FIG. 2, which can control a shape of the high-strength fiber composite, and has a dice capable of controlling impregnation of resin and an amount of resin to be applied to the high-strength fiber bundle.

Hereinbelow is explained a process of fabricating the core 2 in accordance with the first embodiment, by means of the apparatus illustrated in FIG. 2, applying thermoplastic resin to the high-strength fiber bundle. First, the high-strength fiber bundle 5 twisted by a predetermined number is supplied from a creel 7a, and is immersed in molten thermoplastic resin, thermoplastic resin solved into solvent, or emulsion containing thermoplastic resin therein. While the high-strength fiber bundle 5 is being immersed in the thermoplastic resin, the high-strength fiber bundle 5 is squeezed by means of a dice 7f in order for the resin to be impregnated into the high-strength fiber bundle 5. Then, the high-strength fiber bundle 5 is forced to pass through a dice 7b to remove excessive resin, adjust a diameter and a shape thereof into a desired one, and allow the resin to be further impregnated into the high-strength fiber bundle 5. Thereafter, the high-strength fiber bundle 5 is heated in a heater 7c including a pre-heater 7g to remove the solvent to be dried, resulting in that the thermoplastic resin is cured. Thus, there is completed the core 2 comprised of the high-strength fiber bundle 5 to which the thermoplastic resin (a stiffening agent) is applied. The high-strength fiber composite comprised of the core 2 is stored, being kept elongate, in such a condition that the high-strength fiber composite is wound around a drum 7e. After a construction in which the high-strength fiber composite is used has been determined, the high-strength fiber composite is cut into a certain length. As an alternative, the fabricated high-strength fiber composite is cut into a certain length for storage without being wound around a drum.

In the above-mentioned process, after the twisted high-strength fiber bundle was wound around a drum, the drum is attached to a creel for application of the resin to the high-strength fiber bundle. As an alternative, after the non-twisted high-strength fiber bundle was twisted, the resin may be applied to the high-strength fiber bundle without winding high-strength fiber bundle around a drum.

### (Second Embodiment)

Hereinbelow is explained, with reference to FIGs. 3A and 3B, the high-strength fiber composite in accordance with the second embodiment. The high-strength fiber composite is comprised of a core including a high-strength fiber bundle with a constraint wound therearound, the high-strength fiber bundle being integral with the constraint through a stiffening agent in such a condition that the high-strength fiber bundle is kept twisted. Parts or elements illustrated in FIGs. 3A and 3B that correspond to those illustrated in FIG. 1 have been provided with the same reference numerals, and will not be explained.

The high-strength fiber composite 1a illustrated in FIGs. 3A and 3B is comprised of a core 2 comprising a twisted high-strength fiber bundle 5, and a constraint 3 wound around the high-strength fiber bundle 5, where the high-strength fiber bundle 5 and the constraint 3 are stiffened by means of a stiffening agent. Since the structure except the constraint 3 of the high-strength fiber composite 1a is identical with that of the core 2 described in the first embodiment, the structure is not explained.

The constraint 3 bundles high-strength fiber yarns 4 at an outer surface of the high-strength fiber bundle 5 in order to prevent the high-strength fiber bundle 5 from being unbundled. In the second embodiment, the high-strength fiber bundle 5 is constrained with the constraint 3 to keep the high-strength fiber bundle twisted, and a stiffening agent is applied to both the high-strength fiber bundle and the constraint to thereby allow them to be integrated with each other by means of the stiffening agent.

In the high-strength fiber composite 1a in accordance with the second embodiment, the constraint 3 is formed into a braid by winding fibers into a cylindrical braid (a cord). By designing the constraint 3 into a braid shape, it is possible to cover the high-strength fiber bundle with the constraint 3 to such a degree that the high-strength fiber bundle 5 is invisible at an outer surface, and accordingly, the high-strength fiber bundle 5 can be kept bundled, and the constraint acts as a protection layer for protecting the high-strength fiber yarns defining the high-strength fiber bundle 5 covered with the constraint. Thus, the high-strength fiber composite having the above-mentioned structure is used as a brace member or a reinforcement in concrete, it is possible to prevent the high-strength fiber composite from being cut or broken, even if it makes contact with acute materials such as pebbles. Furthermore, since it is no longer necessary for the high-strength fiber composite to additionally include a protection layer, a single high-strength fiber composite can be thinned, and further, fabrication costs can be reduced.

A tensile strength acts on the high-strength fiber bundle 5 constrained with the constraint in a length-wise direction of fibers when excessive resin is squeezed out by means of a dice, after the high-strength fiber bundle 5 was dipped into a resin (a stiffening agent) solution. Since the constraint has a braid structure, spaces surrounded with the fibers are not widened like a knit, but a diameter of a braid is thinned with the spaces being kept closed. Accordingly, adhesion between the constraint and the high-strength fiber bundle can be enhanced without exposure of the high-strength fiber bundle covered with the constraint, which is preferable in the standpoint of a strength of the resultant high-strength fiber composite 1a.

The constraint 3 is designed to have at least a function of preventing the high-strength fiber yarns 4 defining the high-strength fiber bundle 5 from being unbundled. The arrangement of the constraint 3 is not to be limited to a braid illustrated in FIGs. 3A and 3B. Furthermore, it is not always necessary to entirely cover the high-strength fiber bundle with the constraint. A part of the high-strength fiber bundle may not be covered with the constraint.

As examples of arrangement of other constraints, a single constraint may be spirally wound around the high-strength fiber bundle, fibers defining a constraint may be wound around the high-strength fiber bundle to thereby bundle the high-strength fiber yarns by a constraint having a shape of knitted cord and fabricated by knitting coarse cylindrical round braid, or the high-strength fiber yarns may be bundled with a constraint in which fibers listed as the constraint are arranged at a predetermined pitch, as a constraint for bundling the high-strength fiber yarns of the high-strength fiber composite.

In a standpoint of protection of the high-strength fiber bundle, it is preferable to form the constraint in the shape of a braid, and entirely cover the high-strength fiber bundle with the braid-shaped constraint.

The braid-shaped constraint 3 illustrated in FIGs. 3A and 3B may be fabricated by means of an apparatus for fabricating a cord. The high-strength fiber bundle 5 is forced to pass through a center of the apparatus, and the high-strength fiber bundle 5 is covered with the constraint 3 to thereby form the braid. Thus, the braid-shaped constraint 3 is formed on an outer surface of the high-strength fiber bundle 5. The constraint 3 for bundling the high-strength fiber bundle 5 may be twisted or not.

The constraint 3 is preferably soft. As the constraint, there may be used synthetic fiber such as polyamide (nylon and so on), vinylon, polyacryl, polypropylene, vinyl chloride, aramide, cellulose, polyamide, polyester, and polyacetal, recycled fiber such as rayon, half-synthetic fiber such as acetate, and natural fiber such as silk, wool, hemp and cotton. The constraint 3 is comprised preferably of fibers being stable against heat in the case that the constraint is heated during steps of fabricating the high-strength fiber composite or is in an environment of being heated, though dependent on a resistance of the stiffening agent to heat and/or condition of being stiffened. Specifically, it is preferably that the constraint is comprised of polyester fibers, glass fibers or basalt fibers, and it is more preferably that the constraint is comprised of glass fibers. By comprising the constraint of fibers having stability against heat, it is possible to prevent the high-strength fiber yarns and the constraint from being deviated from each other when heated, ensuring accomplishment of a stable tensile strength.

It is preferable in the core 2 that a stiffening agent is impregnated into the high-strength fiber bundle bundled with the constraint to thereby cure the high-strength fiber bundle together with the constraint, in order to intensively bundle the high-strength fiber yarns 4. This ensures that the high-strength fiber bundle and the constraint can be intensively integrated with each other.

The high-strength fiber composite including the intensively integrated core 2 may be formed in a shape of a rod, in which case, the high-strength fiber composite can be stored or carried in a condition of being wound around a drum, or the high-strength fiber composite can be stored or carried after being cut into pieces having a length of a few centimeters to a few meters. In particular, the high-strength fiber composite formed in a shape of a rod can be readily arranged in a narrow groove or inserted into a deep hole, because the high-strength fiber composite does not lose its shape.

In the high-strength fiber composite 1a, the constraint 3 and the stiffening agent act as a protection layer, but the high-strength fiber composite 1a may be designed to further include an actual protection layer (a cylindrical cover comprised of fibers or a resin layer) covering an outer surface of the high-strength fiber composite therewith.

The high-strength fiber composite 1a in accordance with the second embodiment can be fabricated by means of the apparatus used for fabricating the high-strength fiber composite 1. Specifically, the high-strength fiber bundle 5 supplied from the creel 7a is twisted, and then, is fed to an apparatus (not illustrated) for fabricating a cord. Then, the twisted high-strength fiber bundle is fed into a round braid apparatus (not illustrated) to thereby be constrained with a constraint. Thus, there is obtained a high-strength fiber bundle bundled with the constraint. The resultant high-strength fiber bundle bundled with the constraint is immersed in the above-mentioned molten thermoplastic resin, thermoplastic resin solved into solvent, or emulsion containing therein thermoplastic resin. The high-strength fiber composite in accordance with the second embodiment can be obtained by carrying out the steps having been carried out in the above-mentioned first embodiment, except these steps. The high-strength fiber composite in accordance with the second embodiment can be wound around a drum without cutting the high-strength fiber bundle 5, keeping the high-strength fiber composite elongate, and be cut into a certain length after a construction in which the high-strength fiber composite is used has been determined. As an alternative, the high-strength fiber composite may be cut into a certain length without being wound around a drum.

The high-strength fiber bundle 5 may be passed through an apparatus for fabricating a cord, after being twisted, or may be covered with a constraint by means of a round braid apparatus (not illustrated). The resultant high-strength fiber bundle constrained with a constraint is wound around a drum. By equipping the drum to the creel 7a, and carrying out the above-mentioned steps, there can be obtained the high-strength fiber composite in accordance with the second embodiment.

### (Third Embodiment)

The third embodiment which falls under the scope of the present invention is explained hereinbelow with reference to FIG. 4. Parts or elements illustrated in FIG. 4 that correspond to those illustrated in FIGs. 1, 2, 3A and 3B have been provided with the same reference numerals, and will not be explained.

A strand structure 10 illustrated in FIG. 4 is comprised of seven high-strength fiber composites 1a each in accordance with the second embodiment. The centrally arranged high-strength fiber composite 1a (hereinafter, referred to as "high-strength fiber composite 1b") is surrounded by the rest of the high-strength fiber composites 1a (hereinafter, referred to as "high-strength fiber composites 1c").

Since each of the high-strength fiber composites 1a (1b and 1c) has the structure illustrated in FIGs. 3A and 3B, they are not explained in detail. Though not illustrated in FIG. 4, each of the seven high-strength fiber composites 1a (1b and 1c) defining the strand structure 10 is entirely covered at an outer surface thereof with the constraint 3 like a braid.

Though FIG. 4 illustrates the high-strength fiber composites 1a illustrated in FIGs. 3A and 3B as high-strength fiber composites of which the strand structure 10 is comprised, a high-strength fiber composite of which the strand structure 10 is comprised is not to be limited to the high-strength fiber composite 1a, but any high-strength fiber composite may be employed, as long as it falls under the scope of the present invention. In the third embodiment, though both of the high-strength fiber composite 1b and the high-strength fiber composites 1c are identical with the high-strength fiber composite 1a, the high-strength fiber composite 1b and the high-strength fiber composites 1c may be different from each other.

Since the strand structure 10 in accordance with the third embodiment is designed to have a strand construction in which the high-strength fiber composite 1b acting as a core and the six high-strength fiber composites 1c surrounding the high-strength fiber composite 1b are twisted together, it is possible to prevent the strand structure 10 from being unbundled, even if the high-strength fiber composites are not integrated with one another by means of resin. Consequently, the strand structure 10 can have a stable tensile strength. In the case that the strand structure 10 is adhered at an end thereof to a fixation jig, since each of the high-strength fiber composites 1a (1b and 1c) of which the strand structure 10 is comprised is independent from one another, and accordingly, the strand structure 10 has a big surface area, an adhesive for adhering the high-strength fiber composites to the fixation jig can penetrate spaces formed among the high-strength fiber composites, ensuring that an adhesion strength between the fixation jig and the strand structure 10 is enhanced. Furthermore, since the strand structure is comprised of the high-strength fiber composites 1a (1b and 1c) having a tensile strength inherent to a high-strength fiber yarn and being superior in durability against a bending stress, the strand structure can maintain a superior tensile strength even in the case that the strand structure is stretched after having been wound around a drum and hence having been put in a bending stress environment, or that the strand structure is used in a bending stress environment.

A direction in which the high-strength fiber bundles are twisted may be selected from any one of directions identified below. $High-strength fiber bundle \times Strand structure = Direction S \times Direction Z , Direction S \times Direction S , Direction Z \times Direction Z \times Direction S$

If the strand structure is kept to have a fixed diameter, a diameter of strand (a diameter of the high-strength fiber composite) is smaller in the strand structure including a greater number of strands, in which case, though the strand has enhanced flexibility, it is afraid of deterioration in a resistance against being worn out and a resistance against losing its shape.

A number by which the strand structure 10 illustrated in FIG. 4 is twisted is set to be 20 times per a meter. The number is not to be limited to 20 times per a meter, but may be set to be in the range of 1.1 to 50 times per a meter both inclusive in dependence on a purpose. If the number is too small, the high-strength fiber composites 1a are easy to be unbundled into individual high-strength fiber composite. In contrast, if the number is too great, it is afraid that the strand structure has a deteriorated tensile strength. In the case that a number of the high-strength fiber composites is in the range of 7 to 37 both inclusive, the number by which the strand structure 10 is twisted is preferably in the range of 1.5 to 20 times per a meter both inclusive, and more preferably in the range of 2 to 10 times per a meter both inclusive.

The strand structure illustrated in FIG. 4 includes the high-strength fiber composite 1b acting as a core, and the high-strength fiber composites 1c surrounding the high-strength fiber composite 1b, where the high-strength fiber composite 1b and the high-strength fiber composites 1c are twisted together. The strand structure 10 may be fabricated by bundling a necessary number (for instance, 2 to 50 both inclusive) of the high-strength fiber composites, and imparting twist entirely to the thus bundled high-strength fiber composites.

The strand structure 10 can be fabricated by means of a known apparatus. Specifically, the strand structure can be fabricated by winding the high-strength fiber composite 1a around a drum, setting the drum into a creel, and twisting the high-strength fiber composite by a predetermined number by means of a fiber twisting machine, a fiber gathering machine or a fiber collecting machine.

The fabricated strand structure 10 can be wound around a drum without cutting into pieces, keeping the strand structure elongate, and be cut into a certain length after a construction in which the strand structure is used has been determined. As an alternative, the strand structure may be cut into a certain length without being wound around a drum.

A number of the high-strength fiber composites 1a (1b and 1c) of which the strand structure 10 is comprised is seven. However, the number is not to be limited to seven, but is determined in dependence on required performances (in particular, a tensile strength) and an intended use thereof. The number is generally in the range of 2 to 50 both inclusive, and preferably in the range of 7 to 37 both inclusive, though the number is not to be limited to those.

For instance, in the case that the high-strength fiber bundle 5 is comprised of a bundle of 24000 carbon fiber yarns (24k), the strand structure can be preferably used as a brace member, if a number of the high-strength fiber composites of which the strand structure is comprised is in the range of about 2 to about 50 both inclusive.

When a number of the high-strength fiber composites of which the strand structure is comprised is greater than seven, and the high-strength fiber bundles are put one upon another in two or more layers, there may be selected any one of a cross twisting in which the high-strength fiber bundles in each of the layers are twisted by a common twisting angle, and a parallel twisting in which the high-strength fiber bundles are twisted in a single step such that the high-strength fiber bundles in each of the layers are arranged at a common pitch.

In the case that the strand structure is used as a composite including the strand structure and a fixation jig both of which are integrated together, for instance, as a bar to be used in place of a steel bar, a number of the high-strength fiber composites of which the strand structure is comprised is set in the range of about 2 to about 50 both inclusive.

In the case that the high-strength fiber bundle 5 is comprised of a bundle of 12000 carbon fiber yarns (12k) to thereby obtain the strand structure to be used as a wire, a number of the high-strength fiber composites of which the strand structure is comprised is set in the range of about 2 to about 50 both inclusive.

If the strand structure comprised of the high-strength fiber bundles by the above-mentioned number is short of a strength, the strand structure may be designed to include the high-strength fiber bundles by a greater number than the above-mentioned number. From a standpoint of a tensile strength of the strand structure, it is preferable to twist two or more strand structures to thereby define a multi-strand structure in accordance with the fourth embodiment explained hereinbelow.

### (Fourth Embodiment)

The fourth embodiment which falls under the scope of the present invention is explained hereinbelow with reference to FIGs. 5A and 5B. Parts or elements illustrated in FIGs. 5A and 5B that correspond to those illustrated in FIGs. 1 to 4 have been provided with the same reference numerals, and will not be explained.

FIG. 5A is a cross-sectional view of a multi-strand structure 100 in accordance with the fourth embodiment, and FIG. 5B is a side view of the same. The multi-strand structure 100 is comprised of seven strand structures 10 in accordance with the third embodiment. A centrally arranged single strand structure 10a (hereinafter, referred to as "core strand 10a") is surrounded by the rest of strand structures 10b, that is, the six strand structures 10b. Specifically, the multi-strand structure 100 has a strand construction in which the core strand 10a and the six strand structures 10b surrounding the core strand 10a therewith are twisted together, and furthermore, since the strand structures 10 of which the multi-strand structure 100 is comprised have high performances derived from the high-strength fiber composites 1a, the strand structures can have a strength more stable than the same of the seven strand structures 10 merely bundled together. Furthermore, as mentioned earlier, the strand structure 10 is comprised of the seven high-strength fiber composites 1a each entirely covered at an outer surface thereof with the constraint 3 arranged in a shape of a braid, and thus, the constraint 3 arranged in a shape of a braid acts as a protection layer for the high-strength fiber bundles 5 defining the high-strength fiber composite 1a.

Thus, the multi-strand structure is useful as a member to be used in place of a reinforcement steel, or as a rod such as a tension member to be used in place of a PC steel wire, and is particularly useful to a case that a high tensile strength is required.

Though the multi-strand structure 100 is comprised of the strand structures 10, elements for defining the multi-strand structure are not to be limited to the strand structures 10, but may be other strand structures such as the strand structure in accordance with the third embodiment.

A number of the strand structures 10 of which the multi-strand structure 100 is comprised is seven. However, the number is not to be limited to seven, but is determined in dependence on required performances (in particular, a tensile strength) and an intended use thereof. The number is generally in the range of 2 to 40 both inclusive, and preferably in the range of 7 to 37 both inclusive, because it may be difficult to twist the strand structures by a predetermined pitch, if a number of the strand structures is greater than forty.

A number by which the multi-strand structure 100 is twisted is determined in dependence on required performances (in particular, a tensile strength) and an intended use thereof.

A number by which the multi-strand structure 100 is twisted is preferably in the range of 0.3 to 30 times per a meter both inclusive, and is preferably in the range of 0.5 to 15 times per a meter both inclusive in the case that the multi-strand structure 100 includes the strand structures 10 by a number of 7 to 37 both inclusive.

Though the multi-strand structure 100 illustrated in FIGs. 5A and 5B is designed to have a strand construction in which the core strand 10a and the strand structures 10b surrounding the core strand 10a therewith are twisted together, the multi-strand structure 100 may be designed to have a structure in which a necessary number (for instance, 2 to 50) of the strand structures 10 is bundled, and the thus bundled strand structures are twisted to thereby define a multi-strand structure having no core strand.

The multi-strand structure 100 can be fabricated by means of a known apparatus such as a fiber twisting machine, a fiber gathering machine and a fiber collecting machine. Specifically, the multi-strand structure can be fabricated by twisting the strand structures 10 by a predetermined number. The fabricated multi-strand structure 100 can be wound around a drum without cutting into pieces, keeping the multi-strand structure elongate, and be cut into a certain length after a construction in which the multi-strand structure is used has been determined. As an alternative, the multi-strand structure may be cut into a certain length without being wound around a drum.

While the present invention has been described in connection with the preferred embodiments with reference to the drawings, it is to be understood that the embodiments are just examples of the present invention, and the present invention includes all alternatives, modifications and equivalents as can be included within the scope of the subject matter of the present invention, as defined by the appended claims.

### EXAMPLES

Hereinbelow the above embodiments are explained in further detail with reference to examples, but it is to be understood that the scope of the present invention is not to be limited to those specific examples, unless the scope of the present invention is not changed.

### Example 1: High-strength fiber composite

The 24K carbon fiber bundle was constrained at an outer surface thereof entirely with polyester fibers in a shape of a braid by means of a cord fabricating apparatus (24-beating machine) through a process of 8-beat grain beating, in which as a twisted high-strength fiber bundle was used a single 24K carbon fiber bundle (PAN carbon fibers commercially available from Toray Industries, Inc., T700SC) having been twisted by 30 times per a meter in a S-direction, and as a constraint was used polyester fibers (a polyester fiber bundle having 1100 decitex). A ratio with which the carbon fiber bundle was covered at an outer surface thereof with the constraint was almost 100%, and hence, the carbon fiber bundle covered with the constraint was invisible.

Then, the solution (viscosity: 100 mPa-s, B-type viscosity meter, Rotor No. 20, 12 rpm. TVB-15 type viscosity meter commercially available from Toki Sangyo Co., Ltd) containing ingredients identified below was applied to the constrained carbon fiber bundle at 20 degrees centigrade by means of the apparatus illustrated in FIG. 2.

Polymerization type thermoplastic epoxy resin (DENATITE TPEP-AA-MEK-05B commercially available from Nagase ChemteX Corporation): 100 mass parts
Curing agent (XNH6850RIN-K commercially available from Nagase ChemteX Corporation): 6.5 mass parts
Methylethylketone (MEK): 1.6 mass parts
Then, the carbon fiber bundle was heated (150 degrees centigrade, 20 minutes) to polymerize the above-mentioned polymerization type thermoplastic epoxy resin, resulting in that there was fabricated the high-strength fiber composite in accordance with Example 1, comprised of a core including the twisted carbon fiber bundle and the constraint, both being integrated with each other through thermoplastic epoxy resin (a stiffening agent). FIG. 6 is a photograph showing an appearance of the high-strength fiber composite in accordance with Example 1. The thus fabricated high-strength fiber composite in accordance with Example 1 had a diameter of 2.0 mm (measured with calipers).

The high-strength fiber composite in accordance with Example 1 was wound at a room temperature around a drum having a diameter of 50 cm. The high-strength fiber composite could be smoothly wound without being flexed.

### Example 2: High-strength fiber composite

A high-strength fiber composite in accordance with Example 2 was fabricated in the same way as that of Example 1 except that vinylon fibers (vinylon fiber having 1100 decitex) was used in place of polyester fibers (polyester fiber having 1100 decitex).

A bundle of the thus fabricated ten high-strength fiber composites was wound at a room temperature around drums having diameters of 60 centimeters and 50 centimeters, respectively, and then, was aged by a month. Then, the high-strength fiber composites having been aged by a month were cut into pieces having a length of 60 centimeters. Ten high-strength fiber composites were bundled, and then, were inserted through an end thereof into a threaded steel pipe (a length of 120 mm, an inner diameter of 14 mm, an outer diameter of 20 mm). Then, the high-strength fiber composites were fixed in the steel pipes by means of urethane adhesive (commercially available from CEMEDINE CO., LTD., UM890 Kai 1, a main agent: 1 mass part, and a curing agent: 2 mass parts). Then, a tensile strength of the resultant was measured by means of a tensile tester, AG-100kN plus commercially available from SHIMADZU CORPORATION, in accordance with JIS K7165, in which a test piece was A-type, a test speed was 2 mm per a minute, and a jig used for a round rod, was formed with V-shaped grooves extending in parallel with one another. Furthermore, the bundle having been not wound around a drum, and having been aged in a condition of being straight was also measured with respect to a tensile strength.

The measured tensile strength were as follows.
Not wound around a drum: 41.7 kN
Wound around a drum having a diameter of 50 cm: 42.0 kN
Wound around a drum having a diameter of 60 cm: 44.9 kN
Reduction in a tensile strength was not found in the bundles having been wound around a drum for aging.

### Example 3: Strand structure

The high-strength fiber composites in accordance with Example 1, wound around a drum, were bundled by ten. While being heated at 120 degrees centigrade, the bundled ten high-strength fiber composites were twisted in a Z-direction at 20 times per a meter. The thus twisted ten high-strength fiber composites was wound at a room temperature around a drum having a diameter of 70 cm. Thus, there was fabricated the strand structure in accordance with Example 3. The thus fabricated strand structure in accordance with Example 3 had a structure having no high-strength fiber composite acting as a core. FIG. 7 is a photograph showing an appearance of the strand structure in accordance with Example 3.

The thus fabricated elongate strand structure was cut into rods each having a length of 2 m. The rods were inserted through an end thereof into a threaded steel pipe (a length of 120 mm, an inner diameter of 14 mm, an outer diameter of 20 mm). Then, the rods were fixed in the steel pipes by means of urethane adhesive (commercially available from CEMEDINE CO., LTD., UM890 Kai 1, a main agent: 1 mass part, and a curing agent: 2 mass parts). Then, a bending tensile strength of the strand structure in accordance with Example 3 was measured by means of a bending tensile strength evaluation machine (commercially available from TOKYO TESTING MACHINE CO., LTD., RAT100DE-S) in accordance with JSCE-E532-1995. R portions having been used in the bending tensile strength test had diameters of 300 mm and 500 mm. The test was carried out at a speed in the range of 100 to 500 N/mm² both inclusive. A bending angle was 180 degrees.

The bending tensile strength was 66 kN for the R portion of 300 mm, and 66 kN for the R portion of 500 mm, both being superior tensile strength. When the rods were attached to the jigs having the above-mentioned diameters, the rods were not heated, but were attached to the jigs at a room temperature.

### Example 4: Strand structure

The high-strength fiber composites in accordance with Example 1 were prepared by seven. One of the seven high-strength fiber composites was determined to be a core. While being heated at 120 degrees centigrade, the seven high-strength fiber composites in which the core high-strength fiber composite was surrounded by the other six high-strength fiber composites were twisted in a Z-direction by 5 times per a meter to thereby obtain the strand structure in accordance with Example 4. FIG. 8 is a photograph showing an appearance of the resultant strand structure.

### Example 5: Multi-strand structure

The high-strength fiber composites in accordance with Example 1 were prepared by thirty seven. While being heated at 120 degrees centigrade, the 37 high-strength fiber composites were twisted in a S-direction by 8 times per a meter to thereby obtain the strand structure having a four-layered structure of 1×6×12×18. Then, the thus fabricated strand structures were prepared by seven such that one of the strand structures acted as a core and the other six strand structures surrounded the strand structure acting as a core. While being heated at 120 degrees centigrade, the seven strand structures were twisted in a Z-direction by 5 times per a meter to thereby obtain the strand structure in accordance with Example 5. FIG. 9 is a photograph showing an appearance of the strand structure in accordance with Example 5.

### Comparison Example 1

There was fabricated the high-strength fiber composite in accordance with Comparison Example 1 in the same way as Example 1 except that a single non-twisted 24K carbon fiber bundle (PAN carbon fiber commercially available from Toray Industries, Inc., T700SC) was used as a high-strength fiber bundle. A bending tensile strength test was carried out to the high-strength fiber composite in accordance with Comparison Example 1 in the same way as Example 3. Attaching the high-strength fiber composites to an R portion of 300 mm and an R portion of 500 mm, respectively, the high-strength fiber composites were broken.

### Comparison Example 2

The ten high-strength fiber composites each in accordance with Comparison Example 1 were bundled without being twisted as an example analogous to the strand structure in accordance with Example 3. A bending tensile strength test was carried out to the ten high-strength fiber composites in the same way as Example 3. When the ten high-strength fiber composites were attached to an R portion of 500 mm, the ten high-strength fiber composites were broken.

### INDUSTRIAL APPLICABILITY

The strand structure, and the multi-strand structure all in accordance with the present invention can sufficiently have mechanical performances such as a tensile strength and an elastic modulus inherent to high-strength fiber yarn such as carbon fiber yarn, and accordingly, are applicable to various industrial fields such as civil engineering works, construction, vessel, mining and fishery, and are industrially promising.

## Claims

1. A strand structure (10) including a strand construction comprised of two or more twisted high-strength fiber composites (1) whereby each of the twisted high-strength fiber composites includes a core (2) comprised of a bundle (5) of high-strength fiber yarns (4), the bundle (5) being twisted and stiffened with a stiffening agent, **characterized in that** each of the twisted high-strength fiber composites (1) further includes a constraint (3) wound around the bundle (5), the bundle (5) and the constraint (3) being stiffened together with the stiffening agent with the bundle (5) being kept twisted, to define the core (2), **in that** the constraint (3) forms a cylindrical braid of winded fibers, and **in that** the stiffening agent is composed of thermoplastic resin.

2. The strand structure (10) as set forth in claim 1, wherein the high-strength fiber composite is in the shape of a rod.

3. The strand structure (10) as set forth in claim 1 or 2, wherein a number of twisting the bundle (5) is in the range of 2 to 50 times per a meter both inclusive.

4. The strand structure (10) as set forth in any one of claims 1 to 3, wherein the thermoplastic resin is thermoplastic epoxy resin.

5. The strand structure (10) as set forth in claim 4, wherein the thermoplastic epoxy resin is polymerization type thermoplastic epoxy resin.

6. The strand structure (10) as set forth in claim 5, wherein the polymerization type thermoplastic epoxy resin has a straight-chain shaped polymeric structure.

7. The strand structure (10) as set forth in any one of claims 1 to 6, wherein the core (2) has a diameter in the range of 1 to 5 mm both inclusive.

8. The strand structure (10) as set forth in any one of claims 1 to 7, wherein the high-strength fiber yarns (4) include carbon fiber or basalt fiber.

9. The strand structure (10) as set forth in any one of claims 1 to 8, wherein a number of twisting the strand structure (10) is in the range of 1.1 to 50 times per a meter both inclusive.

10. The strand structure (10) as set forth in any one of claims 1 to 9, wherein a number of the high-strength fiber composites defining the strand structure (10) is 2 to 40 both inclusive.

11. A multi-strand structure (100) including a strand construction comprised of two or more twisted strand structures defined in any one of claims 1 to 10.

12. The multi-strand structure (100) as set forth in claim 11, wherein a number of twisting the multi-strand structures (100) is in the range of 0.3 to 30 times per a meter both inclusive.

13. The multi-strand structure (100) as set forth in claim 11 or 12, wherein a number of the strand structures (10) defining the multi-strand structure (100) is in the range of 2 to 40 both inclusive.

## Patentansprüche

1. Strangstruktur (10) mit einer Strangkonstruktion, die aus zwei oder mehr verdrehten hochfesten Faserverbünden (1) besteht, wobei jeder der verdrehten hochfesten Faserverbünde einen Kern (2) umfasst, der aus einem Bündel (5) hochfester Fasergarne (4) besteht, wobei das Bündel (5) verdreht und mit einem Versteifungsmittel versteift ist,
**dadurch gekennzeichnet, dass**
jeder der verdrehten hochfesten Faserverbünde (1) ferner eine um das Bündel (5) gewickelte Beschränkung (3) umfasst, wobei das Bündel (5) und die Beschränkung (3) mit dem Versteifungsmittel zusammen versteift sind und das Bündel (5) verdreht bleibt, um den Kern (2) zu definieren,
dass die Beschränkung (3) ein zylindrisches Geflecht aus gewickelten Fasern bildet und
dass das Versteifungsmittel aus thermoplastischem Harz besteht.

2. Strangstruktur (10) nach Anspruch 1, wobei der hochfeste Faserverbund die Form eines Stabes aufweist.

3. Strangstruktur (10) nach Anspruch 1 oder 2, wobei eine Zahl der Verdrehungen des Bündels (5) im Bereich von einschließlich 2-mal bis einschließlich 50-mal pro Meter liegt.

4. Strangstruktur (10) nach einem der Ansprüche 1 bis 3, wobei das thermoplastische Harz ein thermoplastisches Epoxidharz ist.

5. Strangstruktur (10) nach Anspruch 4, wobei das thermoplastische Epoxidharz ein thermoplastisches Epoxidharz vom Polymerisationstyp ist.

6. Strangstruktur (10) nach Anspruch 5, wobei das thermoplastische Epoxidharz vom Polymerisationstyp eine geradkettig geformte Polymerstruktur aufweist.

7. Strangstruktur (10) nach einem der Ansprüche 1 bis 6, wobei der Kern (2) einen Durchmesser im Bereich von einschließlich 1 bis einschließlich 5 mm aufweist.

8. Strangstruktur (10) nach einem der Ansprüche 1 bis 7, wobei die hochfesten Fasergarne (4) Kohlenstofffaser oder Basaltfaser umfassen.

9. Strangstruktur (10) nach einem der Ansprüche 1 bis 8, wobei eine Zahl der Verdrehungen der Strangstruktur (10) im Bereich von einschließlich 1,1-mal bis einschließlich 50-mal pro Meter liegt.

10. Strangstruktur (10) nach einem der Ansprüche 1 bis 9, wobei eine Zahl der hochfesten Faserverbünde, die die Strangstruktur (10) definieren, einschließlich 2 bis einschließlich 40 beträgt.

11. Mehrfachstrangstruktur (100) mit einer Strangkonstruktion, die aus zwei oder mehr verdrehten Strangstrukturen gemäß einem der Ansprüche 1 bis 10 besteht.

12. Mehrfachstrangstruktur (100) nach Anspruch 11, wobei eine Zahl der Verdrehungen der Mehrfachstrangstrukturen (100) im Bereich von einschließlich 0,3-mal bis einschließlich 30-mal pro Meter liegt.

13. Mehrfachstrangstruktur (100) nach Anspruch 11 oder 12, wobei eine Zahl der Strangstrukturen (10), die die Mehrfachstrangstruktur (100) definieren, im Bereich von einschließlich 2 bis einschließlich 40 liegt.

## Revendications

1. Structure à brins (10) incluant une construction de brins constituée de deux ou plusieurs composites fibreux torsadés de résistance élevée (1),
dans laquelle
chacun des composites fibreux torsadés de résistance élevée inclut une âme (2) constituée d'un faisceau (5) de fils de fibres de résistance élevée (4), le faisceau (5) étant torsadé et renforcé par un agent de renfort, **caractérisée en ce que**
chacun des composites fibreux torsadés de résistance élevée (1) inclut en outre une contrainte (3) enroulée autour du faisceau (5), le faisceau (5) et la contrainte (3) étant renforcés conjointement avec l'agent de renfort avec le faisceau (5) qui est maintenu torsadé afin de définir l'âme (2),
la contrainte (3) forme une tresse cylindrique de fibres enroulées et
l'agent de renfort est composé de résine thermoplastique.

2. Structure à brins (10) selon la revendication 1, dans laquelle le composite fibreux de résistance élevée se présente sous la forme d'une tige.

3. Structure à brins (10) selon la revendication 1 ou 2, dans laquelle un nombre de torsions du faisceau (5) se situe dans la plage de 2 à 50 fois par mètre incluses.

4. Structure à brins (10) selon l'une quelconque des revendications 1 à 3, dans laquelle la résine thermoplastique est une résine époxy thermoplastique.

5. Structure à brins (10) selon la revendication 4, dans laquelle la résine époxy thermoplastique est une résine époxy thermoplastique du type à polymérisation.

6. Structure à brins (10) selon la revendication 5, dans laquelle la résine époxy thermoplastique du type à polymérisation a une structure polymère en forme de chaîne droite.

7. Structure à brins (10) selon l'une quelconque des revendications 1 à 6, dans laquelle l'âme (2) a un diamètre dans la plage de 1 à 5 mm inclus.

8. Structure à brins (10) selon l'une quelconque des revendications 1 à 7, dans laquelle les fils de fibres de résistance élevée (4) incluent des fibres de carbone ou des fibres de basalte.

9. Structure à brins (10) selon l'une quelconque des revendications 1 à 8, dans laquelle un nombre de torsions de la structure à brins (10) se situe dans la plage de 1,1 à 50 fois par mètre incluses.

10. Structure à brins (10) selon l'une quelconque des revendications 1 à 9, dans laquelle un nombre des composites fibreux de résistance élevée définissant la structure à brins (10) est de 2 à 40 inclus.

11. Structure à multibrins (100) incluant une construction de brins constituée de deux ou plusieurs structures à brins torsadées définies selon l'une quelconque des revendications 1 à 10.

12. Structure à multibrins (100) selon la revendication 11, dans laquelle un nombre de torsions des structures à multibrins (100) se situe dans la plage de 0,3 à 30 fois par mètre incluses.

13. Structure à multibrins (100) selon la revendication 11 ou 12, dans laquelle un nombre des structures à brins (10) définissant la structure à multibrins (100) se situe dans la plage de 2 à 40 incluses.
